

## UNITED STATES PATENT OFFICE.

GELLERT ALLEMAN, OF SWARTHMORE, PENNSYLVANIA, ASSIGNOR TO SUN OIL COMPANY, OF PHILADELPHIA, PENNSYLVANIA, A CORPORATION OF NEW JERSEY.

## FATTY ACID AND SOAP DERIVED FROM MINERAL OIL AND PROCESS OF MAKING SAME.

No Drawing.

Application filed July 18, 1925. Serial No. 44,629.

In the manufacture of lubricating oils from crude petroleum, it is customary to subject the same to distillation and then to redistill the distillate, the heavier product remaining in the still being stock adapted for the manufacture of lubricating oil. The second distillate may then be redistilled, the part remaining also being adapted for lubricating stock. Lubricating stock is usually treated with sulfuric or other suitable acid, with agitation, forming an acid sludge, which is drawn off. After the sludge is separated from the lubricating stock, the latter is treated with caustic soda or any other alkali, forming a precipitate, which may be called "soda sludge" or "alkali precipitate", which is drawn off and usually allowed to go to waste.

It is known that this alkali precipitate contains a fatty acid soap or organic acid soap, a large proportion of mineral oil, a considerable body of inert material similar to the fossil resins, which I hereinafter call petroleum resins, some sodium sulfate, and more or less water. It is known to so treat this alkaline precipitate as to eliminate some of the mineral oil, a large part of the water and most of the salts, and to materially reduce the percentage of mineral oil. However, no process has ever been devised to effect an absolute, or even a substantial, elimination of the mineral oil, except the process set forth in my application filed February 6, 1924, Serial No. 691,022; nor has any process been devised to separate the petroleum resins.

In other words, a mineral oil derivative soap that is miscible in all proportions with water or mineral oil, that is not a sulfonic acid soap or a naphthenic acid soap and is adapted to undergo the character of hydrolytic decomposition that occurs with soaps of animal or vegetable origin, that is distinguishable from soaps of animal or vegetable origin in that it contains a substantial proportion of mineral oil and petroleum resins and a minute percentage (say .02 per cent) of sulfur, is known (see Maitland Patents 1,425,882 and 1,425,884); but no such product is known that is also devoid of both mineral oil and petroleum resins; and no such product is known that is devoid of mineral oil except the product set forth in my said application.

So, also, it is known to provide a saponifiable mineral oil derivative, or "fatty acid," that is not a sulfonic or naphthenic acid, and which is a liquid practically odorless, insoluble in water and does not become rancid, and which is saponifiable and when saponified is soluble or emulsifiable in all proportions with water and mineral oil and is adapted to undergo the character of hydrolytic decomposition that occurs with soaps of animal and vegetable oil, and which is distinguishable from soaps of animal or vegetable origin in that it contains a substantial proportion of mineral oil and petroleum resins as well as a minute percentage of sulfur (see Maitland patents aforesaid); but no such product is known that is also devoid of both mineral oil and petroleum resins; and no such product is known that is devoid of mineral oil except the product set forth in my said application.

The object of my invention is to isolate the above described fatty acid and soap derived from mineral oil; or, more accurately stated, to produce a fatty acid and a soap having the characteristics specified above as characterizing known fatty acids and soaps but which is substantially devoid of both mineral oil and petroleum resins. Such isolated fatty acid product, as might be conjectured, I found to be a mixture of acids. The preponderating proportion of these fatty acids have certain compositions and properties which, combined, characterize no known isolated fatty acid derived from any source whatever.

In practicing my process, I may start with any composition derived from mineral oil and containing soap, petroleum resins and mineral oil, such as the alkali precipitate hereinbefore mentioned or the product of the Maitland patents specified. In giving a specific example of the process, it will be understood that the statements therein contained as to the precise details of treatment are predicated upon the treatment of a composition having definite proportions of certain ingredients and produced in the above described treatment of lubricating oil stock derived from Texas oil. It will also be understood that even with this particular crude petroleum, different distillation processes, and even variations in the same distillation proc-

ess, as well as variations in the crude oil, would yield alkali precipitates of varied compositions and characteristics, making advisable some variation from the specific example 5 of the process herein given, in order to secure the elimination of the mineral oil and petroleum resins to the highest degree. The skilled operator, however, can readily adjust the factors to secure the main results sought, namely, 10 the substantially complete elimination of the mineral oil and petroleum resins.

A typical soap emulsion (e. g., alkali precipitate or soda sludge) from which I have succeeded in eliminating the mineral oil and 15 petroleum resins, is as follows:

|                         | Per cent. |
|-------------------------|-----------|
| Soap                    | 11.6      |
| Petroleum resins        | 17.1      |
| Mineral lubricating oil | 46.       |
| 20 Sodium sulfate       | 2.3       |
| Water                   | 23.       |

The soap, oil, and water emulsion, or colloidal suspension, contains particles or droplets which are positively charged. If this 25 mixture is treated with gasoline, practically no separation takes place, except after very long standing. If, however, a small amount of lithium sulfate, sodium sulfate or potassium sulfate, or a small amount of lithium 30 chloride, sodium chloride, or potassium chloride is added to the suspension or emulsion in gasoline, an immediate separation takes place. The sulfates are found to be superior to the chlorides, the double negative charge 35 on the sulfate ion being more effective than the single negative charge on the chloride ion in neutralizing and precipitating the positively charged emulsion particles. Lithium salts are superior to sodium salts, and sodium 40 salts superior to those of potassium. This is a function of surface tension—lithium increasing surface tension more than sodium or potassium, and hence tending to break the emulsion more readily. From a commercial 45 standpoint, sodium chloride (common salt), because of its abundance and low cost, seems to be the most desirable substance to effect the separation of the gasoline and oil, with dissolved resins, from the soap, water and a 50 minor proportion of resins. A saturated solution of the salt is used, being added to the amount of 10 per cent of the total volume. The salt solution may be added before the introduction of the gasoline or it may be 55 added after the gasoline has been distilled into the soap-oil-water emulsion. Instead of using a saturated solution of salt in water, solid sodium chloride (salt) may be added.

It is best to allow the gasoline to enter the 60 crude soap tank, at the bottom, as a vapor. This stirs the mixture, and probably also aids in neutralizing the electrical charges on the suspended colloidal particles. Larger surfaces are exposed to the gasoline, in this manner.

The apparatus employed is conveniently arranged as follows: An upright, cylindrical container is employed to hold the oil-soap-water emulsion, which should fill the container to about one-third its capacity. This 70 is conveniently connected to a gasoline still. The bottom of the first mentioned container should be above the level of the gasoline still. Vapors of gasoline are passed through appropriate pipes, from the still, to the bottom 75 of the container holding the soap-oil-water emulsion. To the emulsion is added a saturated solution of common salt, equivalent in volume to about one-tenth of the soap-oil-gasoline emulsion. Gasoline vapor is introduced at the bottom until the container is almost filled by the condensed gasoline. The introduction of gasoline into this container is then discontinued and the mixture allowed 80 to separate. The gasoline-oil layer on top is siphoned back into the gasoline still and the process repeated. After about three extractions, the soap-water solution which remains in the bottom of the container is substantially 85 free of mineral oil, but contains the petroleum resins that have not been dissolved by the gasoline.

The partially purified soap contains the original sulfur compounds, wholly or principally sodium sulfate, which were in the crude 90 soap. These can be largely removed by known methods if their removal be desirable. For example, the soap solution may be concentrated by first evaporating some of the water (to expedite the operation) and then cooling in order to separate the soap from the sodium sulfate, which remains in solution in the water. The separation begins to take place at about 5° C. and is hastened by lower temperatures. The sodium sulfate 100 remains in solution in the water.

The soap has the characteristics hereinbefore described as characterizing a known product, i. e. that of the Maitland patent specified, but has the further characteristic 110 that it is devoid of mineral oil and of the major part of the resins. If it is desired to convert the soaps into fatty acids it may be so converted by means effective to convert other soaps into fatty acids, as, for example, 115 by decomposing the soap with sulfuric, hydrochloric or other mineral acids. These fatty acids have an acid number of about 103.5. (The original crude soap before treatment yields fatty acids having an acid 120 number of 30.)

The fatty acids are now subjected to distillation at an absolute pressure of 4 mm. of mercury yielding distillates which are free from resins. Up to a temperature of 180° C. a fraction is obtained having an acid number 125 of 187.06. The next fraction boiling off between 180° and 190° C. has an acid number of 174.4. The next fraction boiling off between 190° and 200° C. has an acid number 130

of 160. The residue, containing most of the resins, present before distillation, has an acid number of 61.

Any of these fractions may be, of course, 5 saponified by the addition of any agent adapted to saponify fatty acids. If the fatty acid having an acid number of 103.5 is so treated, it of course, produces a soap the same as that from which the fatty acid was directly 10 derived by decomposition with a mineral acid.

My improved fatty acids differ from ordinary fatty acids of animal or vegetable origin having chemical compositions and molecular 15 weights approximating those of my improved fatty acids in that they are liquid at ordinary temperatures and solidify only at very low temperatures, differ in refractive index and by their degree of volatility (distilling temperature under a vacuum), and do not "dry" or harden when exposed to air but remain sticky or "tacky" indefinitely. At any rate, they have been exposed to observation for a period of eighteen months and 25 still retain this quality.

In order to more particularly differentiate my improved fatty acids from known fatty acids, the following more specific information regarding the compositions, qualities, 30 and properties of the same are given.

1. A predominating proportion of the acids belong to the series  $C_nH_{2n-4}O_2$  and  $C_nH_{2n-6}O_2$ . One acid out of eleven that have been isolated from the mixture of acids 35 seems to belong to the series  $C_nH_{2n-8}O_2$ .

2. They do not absorb oxygen from the air, and do not "dry", or harden.

3. They have an extremely low melting point (below minus 30° C.).

4. They are extremely viscous at low temperatures and will not flow at 0° C.

5. The salts of all the acids are soluble in gasoline, in ether, and in carbon tetrachloride. The lithium, ammonium, potassium, sodium, and magnesium salts are soluble in 45 water.

6. The acids cannot be distilled at ordinary atmospheric pressure without decomposition.

7. At an absolute pressure of 4 millimeters 50 of mercury, the acids volatilize at temperatures ranging between about 160° C. and 245° C.

8. They have an extremely high refractive index. This ranges between 1.48563 and 55 1.49654. Only two of these acids have a refractive index below 1.49, and only one has a refractive index below 1.48968.

9. They are not volatile with steam; that is, when the materials are heated to a temperature above the boiling point of water but to a temperature below the point at which they will volatilize, and steam is passed through the materials, at the bottom of the container, the fatty acids will not pass over 60 with the steam.

10. Their carbon content ranges from  $C_{16}$  to  $C_{25}$ ; that is, there are from 16 to 25 carbon atoms in a molecule of the acid.

11. Their molecular weight ranges from 70 about 250 to about 376.

12. The saponification numbers obtained indicate that there is but one carboxyl group present.

13. They are not naphthenic acids, which latter belong to the series  $C_nH_{2n-2}O_2$ . 75

14. They do not give the reactions of ketonic acids.

In place of using gasoline in the manner described, I may use any light hydrocarbon, whether derived from petroleum or other sources, such as a benzol distillate from coal tar. 80

It is not my intention, however, to limit the product herein claimed to a product produced by the described process, inasmuch as 85 other methods of producing the fatty acids described may be devised. The described method, however, is particularly advantageous, particularly in respect to its simplicity and economy, and is entirely efficient to effect the desired isolation of the fatty acid soap, from which all mineral oil and petroleum resins may be practically completely eliminated by practicing the described process in a thorough and careful manner. 90

Where, in the claims, I refer to soap or fatty acid substantially free of resins, I do not mean to be confined to a product from which the resins are necessarily completely eliminated. The fact that resins are present 100 in the residue from the distillation indicates their presence, in small proportion, in the fatty acids before distillation. It is obvious that the advantages of my new product are present, to a substantial degree, even though the original content of resins is very greatly reduced rather than absolutely eliminated.

Having now fully described my invention, what I claim and desire to protect by Letters Patent is:

1. As a new product, a mixture of fatty acids derived from mineral oil, the same being insoluble in water and readily saponifiable, and when saponified being miscible in 115 all proportions with mineral oil and water and when mixed with oil and water forming a homogeneous emulsion and having essential characteristics of soaps of animal or vegetable origin in that it forms with water a similar emulsion and undergoes the same character of hydrolytic decomposition; the fatty acids being distinguishable from other saponifiable derivatives of mineral oil in that in addition to the characteristics specified they are substantially free of mineral oil and petroleum resins, and being distinguishable from fatty acids of animal or vegetable origin in that they have a melting range below minus 30° C. 120

2. As a new product, a mixture of fatty 125 acids derived from mineral oil, the same being insoluble in water and readily saponifiable, and when saponified being miscible in all proportions with mineral oil and water and when mixed with oil and water forming a homogeneous emulsion and having essential characteristics of soaps of animal or vegetable origin in that it forms with water a similar emulsion and undergoes the same character of hydrolytic decomposition; the fatty acids being distinguishable from other saponifiable derivatives of mineral oil in that in addition to the characteristics specified they are substantially free of mineral oil and petroleum resins, and being distinguishable from fatty acids of animal or vegetable origin in that they have a melting range below minus 30° C. 130

acids derived from mineral oil, the same being substantially free from petroleum resins and mineral oil, and a preponderating proportion of which have the generic formulæ 5  $C_nH_{2n-4}O_2$  and  $C_nH_{2n-6}O_2$  and a melting range below minus 30° C.

3. As a new product, a mixture of fatty acids derived from mineral oil, the same being substantially free from petroleum resins 10 and mineral oil, and a preponderating proportion of which have the generic formulæ  $C_nH_{2n-4}O_2$  and  $C_nH_{2n-6}O_2$  and a melting range below minus 30° C., do not absorb oxygen from the air, cannot be distilled at atmospheric pressure without decomposition, volatilize at an absolute pressure of four millimeters mercury at temperatures ranging between about 160° C. and about 245° C., have refractive indices mostly above 1.49, 15 have carbon contents the molecules of which contain from 16 to 25 carbon atoms and molecular weights ranging from about 250 to about 376.

4. As a new product, a derivative from 25 mineral oil, the same being a soap miscible in all proportions with water and mineral oil, and when mixed with mineral oil and water forming a homogeneous emulsion, and having essential characteristics of soaps of animal and vegetable origin in that it forms 30 with water a similar emulsion and undergoes the same character of hydrolytic decomposition; the new product being distinguishable from soaps of animal or vegetable origin 35 in that the fatty acids from which the soap is derived have a melting range of below minus 30° C. and being distinguishable from other soaps derived from mineral oil in that in addition to the characteristics specified it 40 is substantially free of both mineral oil and petroleum resins.

5. As a new product, a mixture of fatty acids derived from mineral oil, the same being insoluble in water and readily saponifiable, and when saponified being miscible in 45 all proportions with mineral oil and water and when mixed with oil and water forming a homogeneous emulsion and having essential characteristics of soaps of animal or vegetable origin in that it forms with water a similar emulsion and undergoes the same character of hydrolytic decomposition; the fatty acids being distinguishable from other saponifiable derivatives of mineral oil in that 50 in addition to the characteristics specified their acid number is not below about 100, and being distinguishable from fatty acids of animal or vegetable origin in that they have a melting range of below minus 30° C.

6. A soap derived from mineral oil and comprising a saponified mixture of fatty acids having an acid number not below about 100 and a melting range of below minus 30° C., the soap being miscible in all propor-

tions with mineral oil and water and when 65 mixed with oil and water forming a homogeneous emulsion and having essential characteristics of soaps of animal or vegetable origin in that it forms with water a similar emulsion and undergoes the same character 70 of hydrolytic decomposition.

7. As a new product, the hereinbefore described mixture of fatty acids derived from mineral oil, the same being insoluble in water and readily saponifiable, and when 75 saponified being miscible in all proportions with mineral oil and water and when mixed with oil and water forming a homogeneous emulsion and having essential characteristics of soaps of animal or vegetable origin in that it forms with water a similar emulsion and undergoes the same character of hydrolytic decomposition; the fatty acids being distinguishable from other saponifiable derivatives of mineral oil in that in addition to the characteristics specified their acid number is not below about 160, and being distinguishable 80 from fatty acids of animal or vegetable origin in that they have a melting range of be- 85

90 minus 30° C.

8. A soap derived from mineral oil and comprising a saponified mixture of fatty acids having an acid number not below about 160 and a melting range of below minus 30° C., the soap being miscible in all proportions with mineral oil and water and when mixed with oil and water forming a homogeneous emulsion and having essential characteristics of soaps of animal or vegetable origin in that it forms with water a similar 95 emulsion and undergoes the same character of hydrolytic decomposition.

9. As a new product, a mixture of fatty acids derived from mineral oil, a preponderating proportion of which have the generic formulæ  $C_nH_{2n-4}O_2$  and  $C_nH_{2n-6}O_2$  and have a melting range below minus 30 degrees C. and are so nearly pure that their acid number is not below about 100. 105

10. As a new product, a soap comprising 110 a saponified mixture of fatty acids as specified in claim 9.

11. As a new product, a mixture of fatty acids derived from mineral oil, a preponderating proportion of which have the generic formulæ  $C_nH_{2n-4}O_2$  and  $C_nH_{2n-6}O_2$  and having a melting range below minus 30 degrees C., and are so nearly pure that their acid number is not below about 160. 115

12. As a new product, a soap comprising a saponified mixture of fatty acids as specified in claim 11. 120

13. The process of recovering fatty acids from a crude soap emulsion containing soap, mineral oil, petroleum resins and water which comprises adding to the crude soap emulsion a water soluble salt in quantity sufficient to enable the hereinafter specified sep- 125

aration of gasoline to be effected, and passing gasoline vapors into and through the crude soap emulsion and condensing the gasoline on contact therewith, the gasoline dissolving the oil, separating the solution of gasoline and such of the resins as are dissolved therein from the soap, converting the soap into fatty

acids, and by distillation separating the fatty acids from any of the resins that have not dissolved in the gasoline.

10

In testimony of which invention, I have hereunto set my hand, at Swarthmore, Pennsylvania, on this 10th day of July, 1925.

GELLERT ALLEMAN.